

# UNITED STATES PATENT OFFICE.

NATHAN SULZBERGER, OF NEW YORK, N. Y.

## PROCESS OF REDUCING THE SENSITIVENESS OF SILVER COMPOUNDS AND PRODUCTS.

1,356,236.

Specification of Letters Patent. Patented Oct. 19, 1920.

No Drawing. Application filed April 26, 1915, Serial No. 24,148. Renewed September 7, 1920. Serial No. 408,777.

To all whom it may concern:

Be it known that I, NATHAN SULZBERGER, born in New York city, and a citizen of the United States, resident of New York city, in the county and State of New York, have invented new and useful Improvements in Processes of Reducing the Sensitiveness of Silver Compounds and Products, of which the following is a specification.

The means generally employed in photography of producing pictures permanent to the action of light, consist in dissolving out of the developed plate (film, etc.) or out of the print (copy), as in the case of gaslight copying paper and the like, by the aid of sodium thiosulfate the compounds, particularly of silver, as the chlorid and bromid, which are still sensitive to the action of light, after development or printing of the visible picture. This method requires not only great lengths of time, which are necessary in order to effect the complete solution of the sensitive silver salts, still remaining in the material, and also in particular, to wash out the last traces of the thiosulfate, which must be accomplished so as to produce lasting pictures, (directions often speak of from 1-2 hours), but also large amounts of water, making the process inconvenient and in many cases impossible, as particularly, when traveling and in certain climates.

I have found, that these objections, as well as also others, described below and accompanied with the use of sodium thiosulfate, are more or less completely obviated by my method of photography. The same consists in reducing to a larger or smaller extent the sensitiveness toward light of photo-actinic substances, principally the silver compounds, as the silver chlorid and silver bromid, still remaining in the photographic material after development (as in the case of plates, diapositives, films, gaslight papers, etc.) or printing of the picture (as in the case of daylight photo-copying papers, etc.). As will be seen in examples described below, the process requires only a few minutes' time and little water. In fact in instances water has been, for washing purposes, entirely dispensed with, it having been possible to produce pictures by simply using the solutions and (instead of washing out) drying off the one solution, before placing the material in the other.

Since the process does not require the use of sodium thiosulfate, the same is necessarily also free from the disadvantages connected with the use of this salt, which, as is known, often acts also upon the silver contents of the picture, not only dissolving small amounts of such silver, particularly in the presence of air, but particles of the silver picture are also removed in a mechanical way, when the thiosulfate acts as a solvent for the silver, chlorid and bromid. For these reasons particularly, the "unfixed" picture (negative) generally will show more detail than when the same has been treated with thiosulfate.

The following is an example illustrative of the process of my invention as applied to the treatment of a paper containing silver chlorid as its main light sensitive factor, for the production of a picture thereon. However I wish to particularly emphasize that the below described method and quantities employed can be variously modified without leaving the scope of my process and invention.

The paper was developed by means of metol-hydroquinone, the developing agent simply washed out by holding for about half a minute under running water, then placed in a solution of potassium ferrocyanid ( $K_4FeCy_6 + ag.$ ), containing about 15% of the salt. The print can be exposed to the action of light when being placed in this solution for, say, half a minute. After a few minutes the picture was taken out of the solution and dried, after having been again washed for about half a minute in running water. In some cases it may be preferable to use between the developing agent and the ferrocyanid, a bath containing a suitable substance to destroy the action of the developer, as for instance, sodium bisulfite (sulfurous acid, etc.). In either case a picture results, which can be exposed to daylight, without undergoing the change, which such picture will rapidly undergo, when exposed to daylight after only having been treated with the developing agent. I have kept pictures treated in the above way, practically unchanged, for many months. Should it be desirable later on to dissolve out of the picture the silver salts, still remaining in the same and soluble in sodium thiosulfate, this can readily be done. By treating such pictures with various compounds the tone and color of the same can

easily be modified. Thus, pictures which have been desensitized with a ferrocyanid, will take on a brownish coloration when treated, for example, with cupric sulfate, 5 while treatment with a ferric compound will produce a bluish coloration. Rosanilin hydrochlorid produces a pinkish or reddish tone.

As a further example I describe below the 10 preparation of a negative of especial value in connection with X-ray (Roentgen-) photography.

After exposure the plate was developed and, after washing for half a minute in 15 running water, was placed in a bath of sodium bisulfite for a minute or two, again washed as above, and placed in a solution containing less than 1% of palladium-ammonium-protochlorid for a few minutes.

20 After washing as above, the plate was dried, which process can be quickly accomplished, since the palladium compounds have a marked hardening effect upon the plate. The effect in fact of the palladium com- 25 pounds in this respect is so great that such plates have even been placed in boiling water without undergoing apparently any change. Since, therefore such plates may be dried at a higher temperature than can be done when developed and fixed in the ordinary way, an additional advantage is gained (saving of time, etc.) when using this method. The plates, after treatment with the palladium compounds, may be ex- 30 posed to light, the picture remaining clearly visible, especially when holding the same before a brilliant source of light. I have exposed such plates for many weeks to light and was able to clearly view the details in 35 the negative. Although the same still contain silver compounds soluble in thiosulfate, the surgeon can clearly and carefully study the result of his exposure, and even make prints (positives), if so desired. Accord- 40 ing to this process, it is possible to study the negative within about a minute after its development. The same will in many cases also show more details (even in cases where the plate was under-exposed) than after 45 treatment with the thiosulfate. The hardening effect of the palladium compounds also protects the plates, so that the same do not suffer so much from handling. If desirable to dissolve out the silver compounds still 50 soluble in sodium thiosulfate, this can readily be done at convenient time.

Since no developing agent is required, as is the case when working with gas-light paper, the process is still simpler, when 60 copying a negative on day-light paper containing silver chlorid. It is only necessary after printing and washing, to place the picture, for instance, in a solution containing about 15% of potassium ferrocyanid for

a couple of minutes. After washing for a 65 minute the picture is desensitized and can be safely exposed to daylight. The same can be toned, if desired. A treatment with thiosulfate is unnecessary.

All such modifications of the process, 70 which will suggest themselves to those skilled in the art of photography and chemistry shall be considered as coming under the scope of this invention. Also therefore other compounds and mixtures (as for 75 instance with formaldehyde, alum, acids, as for instance, phosphoric, etc.) may be em- ployed which are of a nature adapted to re- duce the sensitiveness of the photo-actinic material, for example, by neutralizing any 80 remaining developer. Instead of potassium ferrocyanid, other soluble ferrocyanids, or derivatives or mixtures thereof, may be used, as well as mixtures in which the soluble ferrocyanids are produced previous to or 85 during the course of the desensitizing proc- ess; as well as other compounds and sub- stances having a similar action.

The term "photo-prints" used in the fol- 90 lowing claims includes reproductions (pos- itive as well as negative) by the action of light with or without the use of a develop- ing agent in a photo-sensitive material con- taining a silver compound.

I claim:

1. The process of reducing the sensitiv- 95 ness toward light of light sensitive silver compounds employed in photography which comprises subjecting such compounds to the action of a solution containing a soluble 100 ferrocyanid.

2. The process of reducing the sensitiv- 105 ness toward light of light sensitive silver compounds employed in photography which comprises subjecting such compounds to the action of a solution containing potassium ferrocyanid.

3. Photo-prints containing light sensitive silver compounds, the sensitiveness toward light of which has been reduced.

4. Photo-prints containing light sensitive silver compounds, the sensitiveness toward light of which has been reduced, and out of which silver compounds may be dissolved by treatment with sodium thiosulfate.

5. Photo-prints, containing light sensitive silver compounds, the sensitiveness of which toward light has been reduced by means of reagents reacting with such silver com- pounds, said photoprints still containing 120 amounts, if only traces, of such employed reagent.

6. Pictures on gaslight paper, containing silver compounds, the sensitiveness of which toward light has been reduced by means of 125 potassium ferrocyanid.

7. Photo-prints containing light sensitive silver compounds, the sensitiveness toward

light of which has been reduced by means of soluble ferrocyanid and still containing amounts, if only traces, of such ferrocyanid and silver compounds soluble in sodium 5 thiosulfate.

8. Toned photo-prints containing silver compounds, the sensitiveness toward light of which has been reduced by means of potassium ferrocyanid, and containing 10 amounts, if only traces, of substances altering the tone of such pictures.

9. The process of reducing the sensitiveness toward light of light sensitive silver compounds employed in gas-light papers

which comprises subjecting such compounds 15 to the action of a solution containing a soluble ferrocyanid.

10. The process of reducing the sensitiveness toward light of light sensitive silver compounds employed in gas-light papers 20 which comprises subjecting such compounds to the action of a solution containing potassium ferrocyanid.

NATHAN SULZBERGER.

Witnesses:

WOLDEMAR HAUPT,  
FRIEDR. CHRISTOPHERS.